

# UNITED STATES PATENT OFFICE.

GUILLIAM H. CLAMER, OF PHILADELPHIA, PENNSYLVANIA.

## IRON-NICKEL-COPPER ALLOY.

1,050,342.

No Drawing.

Specification of Letters Patent.

Patented Jan. 14, 1913.

Application filed July 21, 1910. Serial No. 573,095.

To all whom it may concern:

Be it known that I, GUILLIAM H. CLAMER, a citizen of the United States, residing at Philadelphia, in the county of Philadelphia and State of Pennsylvania, have invented a certain new and useful Iron-Nickel-Copper Alloy, of which the following is a specification.

Objects of the present invention are to 10 effect an economy in the production of nickel-steel of low range, that is, steels in which the nickel is below approximately 8%; to provide low range nickel steel of "pearlitic" structure, in which a portion of 15 the nickel is replaced by copper; to increase the tensile strength of such steel without reduction of the percentage of elongation, and to provide homogeneous iron-copper-nickel alloys having physical properties 20 which adapt them to many uses and purposes in the arts and which are equal to, if not better than those of low range nickel steel.

My invention comprises the partial re- 25 placement of nickel by copper in nickel-steel of low range. Copper to the extent of from  $\frac{1}{2}$  of one per cent. to 2% can be added to nickel-steel of low range without diminishing the physical properties of the steel, 30 and in certain proportions it is even possible by the use of copper to surpass the physical properties of steel containing nickel alone. The basis of comparison in all cases is the amount of the alloying constituent added, 35 i. e., nickel and copper together, being equivalent to nickel alone. By the substitution of a part of the nickel in nickel-steel by copper, the same or greater limit of elasticity and tensile strength are main- 40 tained, without diminishing the ductility. The introduction of copper in place of nickel is advantageous from an economical standpoint, because of the relative differences in price of the two metals. Within this range, it has been found that steel is improved in physical properties by the ad- 45 dition of nickel in increasing degree depend- ing upon the amount of nickel added, until approximately 8% is present. Further ad- 50 ditions of nickel above this percentage are productive of somewhat sudden increase in the tensile strength and limit of elasticity, but this is attained at the expense of greatly

diminished ductility, the steel becoming brit- 55 tle. When, however, nickel is added in still further amount, approaching 25%, the steel again becomes soft and ductile. This is known as steel of high range. Steels with 60 percentages of nickel between these ranges are of no commercial value, owing to their brittleness. These ranges are not, however, sharply defined, and are effected by the car- 65 bon content changes taking place with lower nickel content, as carbon is increased. It is the alloy within the upper percentage range 70 of nickel which is claimed in my co-pending application, No. 513,537. In that application, I have claimed alloys containing cop- 75 per in such amounts that were it added to nickel-steel of low range, as claimed in the present application, or to ordinary carbon-steel or iron, would render them hot short brittle and unmachineable, but the percent- 80 age of copper added in the present invention is such that it has the most desirable effect upon the steel even without the com- 85 bined presence of nickel. I have found that the good qualities to be imparted to steel, both by the addition of copper under 2% or of nickel under 6% can be maintained by 90 the addition of these metals in combination, it being even possible to increase the tensile strength above that which would result from the addition of nickel alone in the same amount as the combined copper and nickel, 95 accomplishing this without any reduction of the percentage of elongation. Carbon may be present in such amount that it will not too seriously affect the ductility, for ex- 100 ample, below .5 of 1%. A small amount of manganese may also be present, and the usual impurities, such as sulfur, phosphorus and silicon, which are present in commercial steel, but naturally these should be kept as low as possible to come within commercial practice. As copper is cheaper than nickel, economy is effected, not only by the nickel displaced by the copper, but also by the smaller percentage of nickel and cop- 105 per required to produce the same physical results. Still further economy may be ef- fected by the use of monel metal, a com- mercial alloy containing approximately 68% nickel, 2% iron and 30% copper. Monel metal is a product made directly from ores carrying nickel and copper, and sells at a

price which is far below the price of refined nickel for nickel contents.

Examples of steels of my invention are as follows:

| 5  | Nickel. | Cop-<br>per. | Car-<br>bon. | Strain<br>per sq. in.<br>in lbs. | Limit of<br>elasticity. | Elonga-<br>tion<br>in 2". | Reduc-<br>tion<br>of area. |
|----|---------|--------------|--------------|----------------------------------|-------------------------|---------------------------|----------------------------|
| 10 | 2.72    | 1.10         | .11          | 83,600                           | 66,300                  | 26.5%                     | 65.4%                      |
|    | 2.00    | .8           | .10          | 75,500                           | 63,700                  | 28.                       | 65.4%                      |

By increasing the amount of carbon to .6%, steel of the composition of the first mentioned in the table, has a tensile strength 15 of 127,500# with elongation 10½% so that from this example, it will be seen that the amount of carbon must be kept within desired limits, for example—approximately below .5 of 1%. Examples given are on un- 20 annealed bars.

What I claim is:

1. Steel containing nickel up to 6% and copper up to 2%. 25
2. Steel containing nickel up to 6% and copper from one-half of one per cent. to 2%.
3. Steel containing nickel up to 6%, copper up to 2% and carbon up to .5 of 1%.
4. Steel containing nickel up to 6%, copper from one-half of one per cent. to 2% and carbon up to .5 of 1%. 30

5. Steel alloyed with 7% of previously prepared alloy of the following approximate composition: nickel 68%, iron 2%, copper 30%.

In testimony whereof I have hereunto signed my name.

GUILLIAM H. CLAMER.

Witnesses:

S. E. PATTERSON,  
K. M. GILLIGAN.